

April 28, 1936.

E. C. DOMM

2,038,548

METHOD OF COATING METAL

Original Filed Jan. 25, 1933



Inventor:  
Elgin Carleton Domm.  
By Dyunforth, Lee, & Tritton & Wilts.  
Atch. 5.

## UNITED STATES PATENT OFFICE

2,038,548

## METHOD OF COATING METAL

Elgin Carleton Domm, Niles, Mich., assignor to  
 National-Standard Company, Niles, Mich., a  
 corporation of Michigan

Original application January 25, 1933, Serial No.  
 653,549. Divided and this application Septem-  
 ber 8, 1934, Serial No. 743,281

6 Claims. (Cl. 91—70)

This invention relates to improvements in method of coating metal.

In the Crapo Patent No. 1,984,335, issued Dec-  
 11, 1934, is described a method of coating a fer-  
 rous article by hot-galvanizing it with zinc, and  
 over that depositing by some other method an  
 additional coating of zinc or a coating of cad-  
 mium.

It has now been discovered that a corrosion-  
 10 resisting coating may be produced which has con-  
 siderable advantage under certain circumstances,  
 particularly with respect to the type of corrosion  
 of which the salt spray is typical, by applying  
 a hot-dipped coating of cadmium, and then elec-  
 15 troplating a coating of zinc thereon.

The invention is particularly applicable to  
 coating strands of wire to be used in reinforcing  
 the bead of the tire. The wire when so used com-  
 monly acts as a tension-member, and is im-  
 20 bedded in a rubber or rubber compound. When  
 so used, the wire is exposed to corrosive and rust-  
 ing agents, particularly to moisture which may  
 seep into the tire.

The drawing shows in diagrammatic form an  
 25 embodiment of my invention.

In accordance with the invention, a metal, for  
 example wire suitable for use in tire beads, is  
 first hot-dipped to provide a coating of cadmium.  
 This may be done, for example, by dipping the  
 30 wire in hot molten cadmium. A coating of zinc  
 is then put over the first coat by electrolysis or  
 by electroplating, preferably by electroplating.

Not only does a double coating applied by the  
 35 above-mentioned method give very good cor-  
 rosion resistance, but it has been discovered that  
 the electro-coat tends to fill in the depressions  
 in the lower cadmium coat and thus produce a  
 uniform and smooth coating. This is wholly  
 unexpected.

If desired, copper or other suitable material  
 40 may be applied over the corrosive-resistant coat-  
 ing in order to increase the adhesiveness of the  
 wire to rubber. It is frequently desirable to  
 apply such a coating when wire is used as a rein-  
 forcement for a tire bead.

The new process herein described is especially  
 useful in procuring a coating of a desired and  
 uniform thickness. In practice, I give the wire  
 a hot coat first, and preferably I wipe this thin.

In the next step, when the coating is put on by  
 electroplating, the operation can be continued  
 to give exactly a desired thickness. At the same  
 time the coating acquires a smooth, uniform  
 character which is free from holes, defects, and  
 the like.

The foregoing description has been given for  
 clearness of understanding only, and no un-  
 necessary limitations are to be understood there-  
 from, but the appended claims should be con-  
 strued as broadly as permissible in view of the  
 prior art.

This application is a division of my co-pending  
 application Serial No. 653,549, filed January 25,  
 1933.

What I regard as new and desire to secure by  
 Letters Patent is:

1. The process of coating a ferrous article which  
 consists in applying to it by the hot-dip process  
 20 a coating of cadmium, and electrodepositing  
 thereon an outer coating substantially wholly of  
 zinc.

2. The method of coating a metal to increase  
 its corrosion resistance comprising first apply-  
 ing to it molten cadmium, and then applying  
 25 a second coating of zinc by electroplating over  
 the first coating.

3. The method of producing a ferrous tire-  
 bead reinforcement wire of uniform corrosion-  
 resistance which comprises first coating a ferrous  
 30 wire with cadmium by the hot-dip process, and  
 then electroplating zinc upon the hot-dipped  
 wire to produce a uniform coating of desired  
 thickness.

4. A coated ferrous article, comprising a fer-  
 rous base having a hot-dipped coating of cadmium  
 thereon, and over that an electrodeposited coat-  
 ing substantially wholly of zinc.

5. A coated ferrous wire, comprising a ferrous  
 base wire having a hot-dipped coating of  
 40 cadmium thereon, and over that an electrode-  
 posited coating substantially wholly of zinc.

6. A coated tire bead wire comprising a ferrous  
 base wire having a hot-dipped coating of cadmium  
 45 thereon, an electrodeposited coating substantially  
 wholly of zinc thereon, and having a coating of  
 rubber vulcanized thereto.

ELGIN CARLETON DOMM.